

## UNITED STATES PATENT OFFICE

2,221,243

## MAGNESIUM BASE ALLOY

John C. McDonald, Midland, Mich., assignor to  
 The Dow Chemical Company, Midland, Mich.,  
 a corporation of Michigan

No Drawing. Application November 13, 1939,  
 Serial No. 304,120

4 Claims. (Cl. 75—168)

The invention relates to magnesium base alloys. It more particularly concerns alloys of this nature having a high degree of formability, coupled with other improved physical properties, such as high tensile and yield strengths.

Magnesium alloys are enjoying increasing use in the structural arts where a light weight metal is highly desirable, such as for use in making large castings, forgings, and the like. However, 10 the use of these alloys in the rolled form to make sheet metal articles requiring forming operations, such as bending, drawing, and the like, has not progressed as rapidly due to the fact that in general alloys of good formability, permitting relatively sharp bends to be made without the article developing external cracks, have inferior characteristics as regards their tensile strength and yield strength.

It is, accordingly, the principal object of the 20 invention to provide a magnesium base alloy which can be made into rolled sheet or the like, possessing a sufficient degree of ductility or formability at ordinary temperatures to be sharply bent, drawn, or otherwise shaped, while having greatly improved tensile and yield strengths.

Other objects and advantages will be apparent as the description of the invention proceeds.

My invention resides in the discovery that a 30 magnesium base alloy composed of from about 0.3 to 12 per cent of silver, 0.05 to 1 per cent of calcium, and 0.1 to 3 per cent of manganese, the balance being substantially all magnesium, is endowed with the afore-mentioned properties. While the property of good formability or ductility, coupled with increased tensile strength and yield strength is manifest over the entire range of composition indicated, I have found that in general the preferred combination of properties, such as the most desirable ductility for forming operations coupled with high tensile strength and greatly increased yield strength, is found in those alloys containing from between about 0.5 to 6.0 per cent of silver, 0.2 to 0.3 per cent of calcium, and 1.0 to 3.0 per cent of manganese. 40 The alloys containing the higher percentages of alloying ingredients, such as from between about 6 to 12 per cent of silver, 0.2 to 0.5 per cent of calcium, and 1.0 to 3.0 per cent of manganese, while not having as good ductility as those in the 50 first mentioned range, do have a much higher yield and tensile strength, and are thus especially suitable for use in casting operations. A preferred alloy having exceptionally good ductility and formability, as well as high tensile and yield strengths, is one containing about 4.0 per

cent of silver, 0.3 per cent of calcium, and 2.0 per cent of manganese.

The improvement in physical properties of my new alloy over that of related alloys is illustrated by the ductility or formability of the above 5 alloy as measured by a conventional bend test. In making the bend test referred to above, a specimen of the alloy is subjected to a 90° bend and the minimum radius of a bend which can be produced without fracture of the specimen at 10 room temperature is noted. The minimum radius thus obtained, expressed in terms of thickness of the specimen being subjected to the test, serves as a measure of the ductility or formability of the specimen. An annealed specimen of 15 my new alloy had a ductility of 2.5 times the thickness of the specimen when subjected to the above test. An annealed specimen of this alloy was also found to have a yield strength of 30,000 pounds per square inch and a tensile strength 20 of 41,000 pounds per square inch. In the cold rolled state the preferred alloy was found to have an elongation of 6 per cent in 2 inches, a yield strength of 45,000 pounds per square inch, and a tensile strength of 49,000 pounds per square 25 inch. Similarly, both ends of the composition range also exhibited correspondingly desirable property values.

The above quaternary alloy clearly has greatly 30 improved properties over those of the closely related ternary alloys. As an illustration, the ternary magnesium-manganese-calcium alloy having similar percentages of manganese and calcium as the above alloy, while having a ductility, as measured by the bend test of 3 times the 35 thickness of the specimen, had in the annealed state a yield and tensile strength of only 21,000 and 35,000 pounds per square inch, respectively. In the cold rolled state this same ternary alloy had a yield and tensile strength of only 31,000 40 and 41,000 pounds per square inch, respectively, with only a 2 per cent elongation in 2 inches. My new alloy also shows improved properties over the related parent ternary magnesium-silver-calcium alloy having the same percentages of 45 silver and calcium as the above illustrated preferred alloy. This ternary alloy, while having a ductility, as measured by the bend test, of 2.5 times the thickness of the specimen, had in the annealed state a yield and tensile strength of 50 only 20,000 and 34,000 pounds per square inch, respectively, while in the cold rolled state the yield and tensile strengths were only 39,000 and 45,000 pounds per square inch, respectively. In addition, this ternary alloy had an elongation of 55

- only 2 per cent in 2 inches. The improvement in properties is also apparent when a comparison is made between my new quaternary alloy and the related ternary magnesium-manganese-silver alloy containing the same percentages of manganese and silver as the preferred alloy illustrated above. The ternary magnesium-manganese-silver alloy had a ductility, as measured by the bend test, of 5 times the thickness of the specimen, and in the annealed state had a yield and tensile strength of only 28,000 and 39,000 pounds per square inch, respectively. In the cold rolled state this ternary alloy had a yield and tensile strength of 44,000 and 50,000 pounds per square inch, but had an elongation of only 4 per cent in 2 inches. The above comparison shows that the combined properties of the new alloy are always superior to those of the related ternary alloys.
- 20 The properties set forth above under the term annealed were obtained by first rolling the alloys at a temperature between about 500° to 700° F. and thereafter annealing them at various temperatures through a range of from 400° to 800° F.
- 25 The properties selected were those of the annealed specimens which exhibited the maximum elongation. The properties set forth under the term cold rolled were obtained by selecting specimens of the alloys which had first been hot rolled
- 30 at a temperature of from 500° to 700° F. to additional rolling in the cold state to bring about a total reduction of from 2 to 10 per cent. The properties selected were those of the cold rolled specimens which showed the greatest tensile and yield strengths, while having at least a 1 per cent elongation in 2 inches.
- 35 While the new alloy is most useful in wrought form, such as sheets, due to its formability char-

acteristics, it may also be suitably used in making castings, forgings, extruded forms, and the like. It is further pointed out that my new alloy is amenable to solution and precipitation heat treatments, which, accordingly, modify its properties.

The new alloy may be compounded in any of the ways known to the art, such as by adding the alloying ingredients to the molten magnesium under a suitable flux. The flux should be substantially free from magnesium chloride if the calcium content of the alloy is to be above 0.3 per cent. In those instances where an alloy is to be compounded containing less than 0.3 per cent of calcium, magnesium chloride may be present in the flux, but in this case it is usually preferable to add the calcium last and without too much stirring or agitation in order to prevent the loss of calcium into the flux.

I claim:

1. A magnesium base alloy containing from 0.3 to 12 per cent of silver, 0.05 to 1 per cent of calcium, and from 0.1 to 3 per cent of manganese, the balance being magnesium.

2. A magnesium base alloy containing from 0.5 to 6 per cent of silver, 0.2 to 0.3 per cent of calcium, and from 1 to 3 per cent of manganese, the balance being magnesium.

3. A magnesium base alloy containing from 6 to 10 per cent of silver, 0.2 to 0.5 per cent of calcium, and from 1 to 3 per cent of manganese, the balance being magnesium.

4. A magnesium base alloy consisting of approximately 4 per cent of silver, 0.3 per cent of calcium, and 2 per cent of manganese, the balance being magnesium.

JOHN C. McDONALD.